

## UNITED STATES PATENT OFFICE

2,426,935

## HECTOGRAPH BLANKET

Irwin Kramsky, Chicago, and Melville J. Holik, Berwyn, Ill., assignors to Ditto, Incorporated, Chicago, Ill., a corporation of West Virginia

No Drawing. Application October 31, 1945,  
Serial No. 625,952

6 Claims. (Cl. 117—35.6)

1

2

The invention relates to composite bonded sheet material and more particularly to hectograph blankets and to methods of preparing the same. Hectograph blankets generally comprise a gelatinous copy mass secured to a flexible backing. In one type of hectograph blanket in commercial use the backing has been secured to the copy mass by means of an intermediate layer of drying oil such as linseed oil. The drying oil may be used by itself or in a lacquer composition. In one type of blanket the backing is coated with a drying oil and then the side remote from the copy mass is coated with a lacquer such as a cellulose ester lacquer which serves as a protective coating. The success of the bond between the copy mass and the drying oil coated backing has been subject to a variety of factors contingent upon (1) degree of oxidation of the drying oils (ageing); (2) humidity and temperature conditions; and (3) quality and concentration of the gelatin and glue used in the copy mass.

An object of this invention is to provide an improved bond between the hectograph copying mass and the intermediate layer containing a drying oil.

A further object is to provide a method for bonding of a gelatin layer to a backing, which method is not so dependent upon degree of oxidation, humidity and temperature and quality and concentration of gelatin as is present with methods hitherto used employing drying oils as bonding agents.

Other objects and advantages of the invention will become apparent as the following detailed description progresses.

We have found a series of compounds which, when added to a gelatin composition such as a hectograph copy mass, facilitate the adherence of the copy mass to a drying oil coated backing and otherwise accomplish the objects of our invention. These compounds consist of water soluble hydroxy aliphatic monoamines and water soluble oxygen containing heterocyclic amines which contain nitrogen in the trivalent form. Suitable compounds include, for example:

- (a) 2-amino-1-butanol
- (b) Mono, di, and triethanolamine
- (c) Mixed isopropanol amines
- (d) Tris (hydroxymethyl) amino methane
- (e) 2-amino, 2-ethyl, 1,3-propanediol
- (f) 2-amino, 2-methyl, 1,3-propanediol
- (g) 2-amino, 2-methyl, 1-propanol
- (h) Diethylaminoethanol
- (i) Morpholine
- (j) Ethyl morpholine

These compounds may be incorporated with all types of gelatin containing compositions for which it is desired to obtain an efficient bond to a backing of paper, cloth, metal or the like, particularly where the backing is coated with a composition consisting of or containing a drying oil such as linseed oil, poppy oil, tung oil and the like. However, our invention is particularly applicable to secure hectograph compositions to paper or cloth backings. These hectograph compositions, as is well known in the art, are gelatin gels containing a major proportion of a relatively non-volatile water soluble material such as glycerin. For example, hectograph blankets generally contain to 1 part by weight of gelatin, 5 to 20 parts by weight of glycerin, and from 1 to 3 parts by weight of water. The water soluble amine may be incorporated in this composition in a proportion of 1% to 50% by weight, preferably from 5% to 25% by weight. Minor proportions of tanning agents based on the gelatin are also incorporated in the mixture. Formaldehyde, aluminum alums, chrome alums and potassium and ammonium dichromates may be used. For example, .001 to .01 of potassium dichromate may be incorporated in the gelatinous mass.

To more clearly set forth the practice in accordance with the invention, and to more specifically point out the nature of the product and process contemplated thereby, several specific, illustrative examples of suitable compositions are hereinafter set forth, it being understood that these examples illustrate several embodiments which have given satisfactory results and are not intended to restrict the invention thereto.

## Example I

|                                       | Parts |
|---------------------------------------|-------|
| 225 bloom gelatin                     | 150   |
| Water                                 | 200   |
| 40 2-amino, 2-methyl, 1,3-propanediol | 15    |
| Glycerin                              | 1800  |

## Example II

|                      | Parts |
|----------------------|-------|
| 45 225 bloom gelatin | 150   |
| Water                | 200   |
| Triethanolamine      | 25    |
| Glycerin             | 1790  |

## Example III

|                      | Parts |
|----------------------|-------|
| 50 225 bloom gelatin | 150   |
| Water                | 200   |
| Aminobutanol         | 25    |
| Glycerin             | 1790  |

55 To prepare the gelatin compositions, the gelatin was first soaked in the aqueous amine solu-

tion, then warmed to 53° C. and added to the glycerin, which has been preheated to 62° C.

While we do not intend to be limited to any theory as to the action of amine compounds, the following explanation is given for the purpose of aiding and understanding our invention:

Assuming a structure for the unsaturated, free fatty acids of the drying oils in the bonding layer to be



upon oxidation, a diperoxide structure represented by the formula:



is formed.

Representing the simplified formula of a hydroxy alkyl monoamine as:



where  $R'$  is an alkyl radical with hydroxyl group and  $R''$ ,  $R'''$  are alkyl or hydroxyalkyl radicals and examining the electronic structure:



where  $\delta$  represents nitrogen electrons and  $\cdot$  represents  $R'$  electrons it may be shown that, being soluble in water,



a hydrated amine of the oxonium type based upon a coordinate link involving 2 covalent hydrogen, called the hydrogen bond, a semi-polar linkage. This linkage is semi-ionic in nature, and its presence is established from the number of covalent bonds in the completed valence shell of the atom. One of the valences of pentavalent nitrogen is an electrovalence different from the other four. The four valences of nitrogen have a tetrahedral spatial arrangement, but the group held by the electrovalence is attracted by the ammonium ion as a unit by virtue of the electrostatic charge without definition of direction. This compound, then, is capable of forming a substantially stable salt attributable to the resonance effect allied with hydrogen bond.

This is believed to react with the peroxide portion of the oxidized unsaturated free fatty acid as follows: the amine hydrate forms an amine oxide hydrate from the peroxide;



this hydrate then forms a partial ether linkage with the ethylenic oxide,



Thus the conversion of trivalent nitrogen makes it possible to form a connecting bridge with the bonding layer. This is substantiated by the fact that pentavalent nitrogen compounds do not perform this function.

Since protein, e. g., gelatin or glue, is a hydrophilic colloid, and the case of a colloidal solution of a more or less linear molecule of high molecular weight, such as gelatin is assumed to be, produces an interlocking network of molecular fibers leaving a high proportion of open liquid-filled spaces which retain their properties of electrical conductivity and diffusivity of solute, it can logically be assumed that groups of a hydrophilic character, such as hydroxyl, will seek out the interstices of water and become imbedded in the colloidal solution. Thus a bridge linking the bonding layer to the protein layer is established between the amine portion of a molecule, and the hydroxy portion of a molecule.

While we have described certain preferred embodiments of our invention, many modifications thereof may be made without departing from the spirit of the invention; and we do not wish to be limited to the detailed examples, formulas, and proportions of ingredients herein set forth, but desire to avail ourselves of all changes within the scope of the appended claims.

We claim:

30 1. A composite sheet comprising a layer of gelatin containing a compound selected from the group consisting of water soluble hydroxy aliphatic monoamines and water soluble oxygen containing heterocyclic monoamines containing nitrogen in a trivalent form; a backing, and an intermediate layer containing a drying oil.

2. A hectograph blanket comprising a backing, a gelatinous copy mass comprising gelatin and containing a compound selected from the group consisting of water soluble hydroxy aliphatic monoamines and water soluble morpholines; and an intermediate bonding layer comprising a drying oil.

3. A hectograph blanket comprising a fibrous backing, a gelatinous copy mass comprising gelatin and containing a compound selected from the group consisting of water soluble hydroxy aliphatic monoamines and water soluble morpholines; and an intermediate bonding layer of linseed oil.

4. A hectograph blanket comprising a backing, a gelatinous copy mass comprising gelatin and containing a hydroxy aliphatic monoamine, and an intermediate bonding layer comprising a drying oil.

5. A hectograph blanket comprising a backing, a gelatinous copy mass comprising gelatin and containing an ethanolamine, and an intermediate bonding layer comprising a drying oil.

6. A hectograph blanket comprising a backing, a gelatinous copy mass comprising gelatin and containing a morpholine; a backing, and an intermediate layer containing a drying oil.

IRWIN KRAMSKY  
MELVILLE J. HOLIK.

#### REFERENCES CITED

The following references are of record in the file of this patent:

70 UNITED STATES PATENTS  
Number Name Date  
1,982,018 Owen Nov. 27, 1934